

# UNITED STATES PATENT OFFICE.

YORK SCHWARTZ, OF HANOVER, GERMANY.

## PHOTOGRAPHIC EMULSION.

962,788.

Specification of Letters Patent. Patented June 28, 1910.

No Drawing.

Application filed May 6, 1907. Serial No. 372,232.

To all whom it may concern:

Be it known that I, YORK SCHWARTZ, a subject of the King of Prussia, and resident of 3 Edenstrasse, Hanover, in the German Empire, have invented a new and useful Photographic Emulsion, of which the following is an exact specification.

The present invention relates to an improved photographic emulsion of the kind set forth in the specification of United States patent granted to York Schwartz No. 710019 dated September 30th, 1902. The emulsion is there indicated as containing an emulsifying agent, silver phosphate, silver chlorate and a silver salt of an organic acid. It has been found that such an emulsion is insufficiently sensitive for some purposes and accordingly the present invention has for its object to modify the emulsion in such a manner as to obtain greatly increased sensitivity. For this purpose in the improved form of the emulsion the proportion of the phosphate used is increased so that it is considerably in excess of that theoretically necessary for the decomposition of the whole of the silver nitrate employed in the preparation of the emulsion.

The preparation of the emulsion is carried out as follows:—In the presence of a colloidal substance, for instance gelatin, an alkaline phosphate, preferably disodium phosphate, is mixed with nitrate of silver, the relative proportion of the phosphate being as above indicated in excess of that necessary for the decomposition of the silver nitrate. It has been found in practice that it is preferable to use double the quantity of phosphate which would ordinarily be necessary to effect this decomposition. To this mixture an oxidizing agent, such as chlorate of potassium, and citric acid or its equivalent are added and if desirable a small quantity of chrome alum may be used for rendering the sensitive surface more resistant.

It is at present impossible to state with certainty what chemical action the various constituents of the mixture have upon one another in forming the emulsion. The chlorate of potassium acts as an oxidizing agent, and the citric acid acts as a solvent for the phosphate, without decomposing the same, as is clearly well known. There is also no doubt that the whole of the silver nitrate is decomposed by the phosphate. The exact nature of the action of the other constituents of the mixture is however not so clearly un-

derstood. In ordinary course if citric acid were brought in contact with the alkaline phosphate the phosphate would be decomposed and a citrate and free phosphoric acid 60 produced. The special conditions of the present case however appear to bring about a further reaction and, although the inventor has hitherto been unable to prove the theory by isolating and analyzing the compound, he has good reasons for believing that a double salt of the form of a phospho-citrate of silver is produced. This compound when acted upon by the developer after the action of light has loosened the cohesion of 70 its constituents appears to be split up into two compounds, one of which during development liberates nascent silver while the other attracts this body, the extent of these actions being proportional to the light action 75 to which each part of the sensitive surface has been subjected. The applicant does not however bind himself to this explanation of the constitution of the emulsion.

Experiments have proved the emulsion to 80 be sufficiently sensitive to enable it to be used not only for contact-printing, but also for enlarging purposes and even for the negative process. While in the former cases the development is carried out "physically" i.e. 85 in acid or neutral solution, chemical development, i. e. in alkaline solution, is preferably used in the latter. Every sort of suitable material, paper, glass, etc., may be coated with the emulsion.

The best developer for this emulsion is a simple aqueous solution of metol. The developers necessary for the development of the emulsion prepared according to the patent above referred to were of rather complicated nature and are entirely dispensed with in the case of the new emulsion.

The pictures developed by means of the aqueous metol-solution show great intensity and brilliancy and very nice tones, and furthermore great durability. By adding sulfite of sodium to the aqueous solution of metol the rapidity of development is so increased that it takes place nearly instantaneously, the development in this case being a 100 chemical one. This method of development is preferably used for the negative process with this emulsion.

### Claims.

1. A photographic emulsion formed by 110 the mixture, with a colloidal substance and silver nitrate, of a quantity of alkaline phos-

phate in considerable excess of that required to decompose the whole of the silver nitrate, with an oxidizing agent and a substance acting as a solvent for the phosphate without 5 decomposing the same.

2. A photographic emulsion formed by the mixture with a colloidal substance and silver nitrate, of a quantity of alkaline phosphate approximately double that required 10 for the decomposition of the whole of the silver nitrate, with an oxidizing agent and a substance acting as a solvent for the phosphate without decomposing the same.
3. A photographic emulsion formed by

the mixture with a colloidal substance and 15 silver nitrate, of a quantity of disodium phosphate approximately double that required for the decomposition of the whole of the silver nitrate, with chlorate of potassium and citric acid, whereby an emulsion is 20 produced having as one of its principal constituents a phospho-citrate compound.

In witness whereof I have hereunto set my hand in the presence of two witnesses.

YORK SCHWARTZ.

Witnesses:

PAUL R. THOMPSON,  
H. T. FULLER.